

Patented Mar. 12, 1940

2,193,090

# UNITED STATES PATENT OFFICE

2,193,090

## COMPOSITE TRANSMISSION LINE

Flint C. Elder, Cleveland Heights, Ohio

No Drawing. Application April 14, 1936,  
Serial No. 74,359

2 Claims. (Cl. 174—132)

The present invention relates to a composite transmission line for use as an overhead power cable and comprises a ferrous metal conductor core having a metal coating alloyed thereto and subsequently cold-worked to provide a yielding point having not less than 90 per cent of the ultimate tensile strength of the material.

An object of the present invention is to provide a composite wire consisting of a ferrous metal core wherein the range of carbon is as low as possible and the manganese content may be of the same range as the carbon content but preferably as low as possible to increase conductivity with a coating of one of the non-ferrous metals of the class electro positive to iron with subsequent cold-working of the composite wire to produce a yielding point substantially that of the ultimate tensile strength of the material.

The present invention resides in coating a carbon steel core wherein the range of carbon should be as low as possible but can extend from .01% to .50% but is preferably in the range between .01% to not over 0.24%. The range of manganese may be the same as the carbon but should be as low as possible in order to increase the conductivity thereof.

This conductor is then provided with an excessive amount of coating of a metal which may be one of the non-ferrous metals of the class which are electro positive to iron in accordance with the method described in applicant's Patent No. 2,049,834. After the required thickness of coating is applied to the conductor, the composite wire is then cold-worked in any suitable manner and in so doing, produces a composite wire having a yield point far greater than any of the known wires used for this purpose today and carry a yield point of not less than

90 per cent of the ultimate tensile strength thereof. By applying an excessive amount of coating onto the conductor before the cold drawing operation, it is possible to produce a high tensile conductor from low carbon steel having a yield point not less than 90 per cent of its ultimate tensile strength so that the conductor, at finished size, will have the prescribed amount of coating.

While I have described one specific embodiment of my invention, it will be understood that I do not wish to be limited exactly thereto, since various modifications may be made without departing from the scope of my invention as defined by the following claims.

1. A conductor comprising a ferrous metal core having a heavy galvanized coating alloyed thereto, said conductor being cold-worked after coating to raise its yield point to not less than 90 per cent of the ultimate tensile strength of said core and to provide a finished coating of an amplitude corresponding to that required on a similar wire but which has been coated subsequent to cold-working.

2. A conductor comprising a ferrous metal core having a heavy galvanized coating alloyed thereto, said ferrous metal core having a carbon content of less than .25 per cent and a manganese content equal to or less than the carbon content, said conductor being cold worked after coating to produce a wire having high tensile strength and a yield point not less than 90 per cent of the ultimate tensile strength of said conductor and a finished coating of an amplitude corresponding to that required on a similar wire but which has been coated subsequent to cold working.

FLINT C. ELDER.